

## UNITED STATES PATENT OFFICE

HARRY H. STOUT, JR., OF NEW YORK, AND WILLIAM H. OSBORN, OF GARRISON, NEW YORK, ASSIGNEES TO COPPER DEOXIDATION CORPORATION, OF NEW YORK, N. Y., A CORPORATION OF NEW YORK

## METHOD OF MAKING BRITTLE CATHODES

No Drawing.

Application filed September 18, 1929. Serial No. 393,575.

This invention relates to a new and improved method for the electrolytic refining of metals.

The principal object of the invention is to provide a method that will produce a copper cathode deposit that is coarsely crystalline and brittle, so that it is easily frangible. This result is achieved by coating the surface against which the copper is to be deposited with a film of material suitable to produce the desired result.

10 The brittle copper deposit can easily be stripped from the coated surface, and reduced to small lumps that can be economically handled in subsequent operations.

A further advantage of the process lies in the savings that can be effected in the operation of the electrolytic process itself.

These and other objects and advantages 20 of the invention will become apparent as the description proceeds.

While preferred methods of carrying out the invention are disclosed herein, it will be understood that various changes may be 25 made in the process without departing from the spirit and scope of the invention as hereinafter set forth and claimed.

In current practice of electrolytic refining of copper the object is to obtain a deposit 30 that is as tough as possible, and several expedients are used to further that purpose. Thus in present multiple systems practice, two important steps are employed. First, small quantities of glue are added to the electrolyte, which has the effect of increasing the degree of adhesiveness or cohesiveness between the deposited crystals and hence making the whole deposit tough. Second, the deposit is made on both sides of a thin, 40 specially prepared electrolytically deposited starting sheet to which the deposit adheres, forming a sheet of double thickness deposition cemented together by the starting sheet. The whole, i. e., deposit plus starting sheet, 45 forming a three-ply heavy cathode, is melted up as one cathode in further treatment.

This system presents certain definite tank room disadvantages, among which may be listed:

50 1st. The expense of making starting sheets.

2nd. The increased power required due to presence of glue which increases the resistance and/or polarization of the electrolyte.

3rd. The increased power to overcome resistance of the loops by which the starting sheets are suspended from the cathode supporting rod and to overcome contact resistance between supporting rod and loop.

4th. The thin starting sheets have a tendency to warp, causing short circuits against the anode with consequent loss of power and increased cost of inspection labor to prevent their forming.

In the present process, it not being necessary to form a tough deposit, glue is preferably omitted from the electrolyte and a relatively heavy blank of hard rolled copper, or other suitable material, replaces the light starting sheet. The blank is reusable and hence is firmly fixed to the cathode supporting rod, eliminating the resistance of cathode suspending loop and loop contacts. Warping is done away with.

In the preferred form the process of this invention is carried out as a multiple process 75 in the following manner:

A. A suitable blank of suitable metal, preferably of hard rolled copper of sufficient thickness to stand the abuse of average handling without denting, bending or warping (approximately  $\frac{1}{8}$ " has been found suitable) is cut to the desired dimensions and firmly attached to the cathode suspending rod so as to eliminate contact resistance at this point.

B. The blank is then coated with a suitable film to produce the desired brittle deposit. A preferred coating is a film of asphalt, which may be conveniently applied by dipping at a suitable temperature, the blank in a solution or emulsion of asphalt. When this emulsion dries it leaves a very thin, transparent film of asphalt with a strong adhering power and high dielectric strength.

C. The blank coated as above is placed in the electrolytic tank and deposit is made. The electrolyte may be of usual composition, except that as explained above glue is preferably omitted. Goulac, or any other similar organic compound ordinarily used to promote

eveness of distribution may be used if desired.

D. When the deposit has reached a suitable thickness, the cathode is lifted from the tank and the deposit stripped from the blank by any preferred means such as rapping the blank with a hammer, stripping with any form of stripping instrument or blade operated either by hand or mechanically, or by 10 any other suitable means.

E. The deposit stripped from the blank is then broken up to desired particle size by shattering on the floor and passing through a grizzly, or by breaking in a trundle barrel, 15 or by any other suitable means.

The blanks are then ready for a repetition of the cycle of coating and deposition.

The copper deposited by this method is so brittle that a 14 day deposit, using 16½ 20 amperes per square foot current density, can easily be broken by the fingers of a bare hand into pieces of approximately ¼ inch in diameter. After breaking up, the particles vary from ⅛ inch up to 1 or more inches in diameter, 25 with very few fine particles, which are to be avoided as tending to cause copper losses in subsequent handling.

It is not the intention to limit the process to any particular theory of operation, but it 30 is believed that the production of the brittle deposit can be explained in the following manner.

In normal electrolytic deposition of copper against a plate or blank the resistance to deposition at the start of current flow is so slight 35 that an almost uniform layer of copper composed of minute interlocked crystals is deposited simultaneously over the entire blank, and as this layer grows out, it forms a tough 40 skin of copper next to the blank. If glue is used in the electrolyte this tough bonding of the cathode crystals will tend to continue throughout deposit. If no glue is used the crystals will tend to adhere less closely to 45 each other as the deposit grows out and the crystals increase in size—and the final result will be a cathode composed of crystals relatively loosely adhering on the electrolyte side of the deposit, but firmly held together by the 50 tough skin formed in the first period of deposition when the crystals, or crystal foci, were still very fine.

In the process of the present invention the coating used places between the blank and 55 the electrolyte a continuous film opposed to the passage of current. As the current pierces this film at relatively separated points copper is deposited and crystals are formed which grow to relatively large size before coming 60 into contact with their neighbors, and hence the crystals never adhere very closely to each other. Obviously too impervious a film will prevent deposit altogether and an insufficiently impervious film will not produce the desired effect. When using a coating substance 65

that is fluid at the temperature of the electrolyte, the coating substance must have a correct balance of the three following factors:

1. *Viscosity of the fluid.*—This controls the thickness of the film when immersed in electrolyte. 70

2. *Power of wetting, or adhering, to the copper blank—and hence preventing displacement of the substance by electrolyte at surface of blank.*—In general the power of hydrocarbons to wet and adhere to the blank 75 is greater with those high in unsaturates and less with those low in unsaturates. The iodine number of an oil is a rough indication of its degree of unsaturation, hence of its 80 wetting power.

3. *Dielectric strength of the filming substance.*—The higher the dielectric strength, other factors being equal, the greater the resistance to current passage. 85

In the case of a coating substance that is solid at the temperature of the electrolyte, such as some waxes, or a thin film of asphalt the first two factors are automatically taken care of, and the degree of resistance of the 90 film is regulated by the amount of coating substance applied. A continuous, solid film of wax of very high dielectric gives a very brittle deposit even when applied very thin.

Corn oil, when used as a coating material, 95 gives a very brittle deposit. This is a highly fluid oil of low viscosity, that forms a thin film, but is of very high wetting power and high dielectric.

On the other hand, a high dielectric cable 100 oil will give a tough deposit. This oil is of medium viscosity and very high dielectric, but it is composed of almost completely saturated hydrocarbons, and hence is of very low wetting or adhering power. 105

Ordinary double distilled rosin oil also 110 gives a fairly tough deposit. This oil is of medium viscosity and good adhering power, but low dielectric.

Among other substances that have been 115 found to yield a brittle deposit when correctly used, the following may be enumerated; linseed oil, sulphonated corn oil, crude fuel oil, cerowax made by the Vacuum Oil Company, superlowax made by the Standard 120 Oil Company of Indiana. The invention contemplates the use of any coating substance that will produce the desired result, and these 125 coating substances may be applied in different conditions, such as in various degrees of solution, in combination with a neutral agent or a beneficial agent, or in an emulsion form where the substances can be emulsified. The coating substances can be applied in the most practical manner, as by dipping, painting, 130 swabbing, spraying, etc.

The power saving of this process over common practice has been found, in comparative runs in a semi-commercial unit, to be approximately 15% of the total power used. This 135

saving and the saving in labor in preparing starting sheets and in inspection against warping, considerably over-balances the cost of copper tie-up in the blanks and the cost of applying coating to the blanks, both necessary with the new process, so that the net saving per ton of cathode produced by the multiple system by the new process is considerable.

10 All cathodes on removal from the electrolyte carry on their surfaces, and between crystal faces, certain impurities which are included in the electrolyte and adhere with it to the copper. Such impurities include slimes 15 suspended in the electrolyte and such compounds as copper, iron and nickel sulphates dissolved in the electrolyte, and also certain arsenic compounds, etc. In the present practice tough cathode sheets are dipped in or 20 sprayed with some solution, usually hot water, to wash off as much as is practicable of these adherent impurities before further treatment.

It has been found that the loosely adhering 25 crystals of brittle cathode deposit are more permeable to the washing action of hot water, or acid or alkaline solutions, or other suitable solutions, than is tough cathode material and that by percolation or agitation of 30 a washing solution through the granular mass of loosely adherent cathode crystals, it is possible to obtain a more thorough degree of washing at less expense than can be done by spraying or dipping of tough cathode 35 sheets.

The economical production of brittle cathode is important in connection with any process of refining where it is desired to bale the cathode into billets for subsequent treatment.

40 Those skilled in the art will recognize that the new process disclosed herein has many advantages, and they will appreciate the fact that the novel features are also applicable to the series process of electrolytic refining. It 45 will also be understood that the process can be applied to the electrolytic deposition of other metals, such as zinc.

We claim:

1. The process of electrolytic deposition of 50 copper which includes coating a blank with a film of asphalt, inserting the blank in a bath of electrolyte and passing an electric current through the electrolyte between the blank and an anode, the asphalt film being 55 of such thickness and properties that copper is deposited against it from the electrolyte in a brittle deposit.

2. That step in the process of electrolytic deposition of copper which comprises dipping a blank in an emulsion of asphalt and subsequently drying the emulsion to cover the blank with a film of asphalt.

3. The process of electrolytic deposition of copper which includes coating a surface upon which the copper is to be deposited with

an embrittling film containing unsaturated hydrocarbons, the embrittling film having such dielectric strength that the current will pierce the film only at points that are separated from each other relatively widely to 70 start building copper crystals, the embrittling film having sufficient wetting power to wet the copper crystals as they are formed, inserting the part carrying the coated surface in a bath of electrolyte, passing an electric current through the electrolyte to the coated surface, thereby depositing a cathode copper mass which has sufficient cohesive strength to remain attached to the coated surface during deposition but which can be 75 readily stripped from the coated surface after deposition, and which is sufficiently brittle to permit its being readily broken up into hunks after it is stripped from the coated surface.

In testimony whereof we affix our signatures.

HARRY H. STOUT, JR.  
WILLIAM H. OSBORN.

90

95

100

105

110

115

120

125

130